

**1**

3,415,669

**BITUMEN COMPOSITIONS AS MOLD COATINGS**  
Edward G. Elste, Jr., Lutherville, Md., assignor to  
Chevron Research Company, San Francisco, Calif.,  
a corporation of Delaware

No Drawing. Continuation-in-part of application Ser. No. 478,982, Aug. 11, 1965. This application July 28, 1967,  
Ser. No. 656,692

5 Claims. (Cl. 117—5.1)

5

10

**ABSTRACT OF THE DISCLOSURE**

Bitumen compositions having high total asphaltene-aromatic components to paraffinic component ratios with 15 high autoignition temperatures for ingot mold coatings.

20

**CROSS-REFERENCES TO RELATED APPLICATIONS**

This application is a continuation-in-part of application Ser. No. 478,982, filed Aug. 11, 1965, now abandoned.

25

**BACKGROUND OF THE INVENTION****Field of the invention**

In order to minimize scabs and other imperfections when forming steel ingots, the ingot mold is coated with various materials. The imperfections in the ingot result because of the great temperature differential between the mold temperature and the molten steel temperature. While the mold temperature may range between about 100° F. and 1200° F., the molten steel will be at least about 2900° F. When pouring the molten steel, splashes will freeze and crystallize onto an uncoated mold surface. These solid splashes having different crystal structure from the major portion of the ingot result in imperfections and irregularities. With a properly coated ingot mold, the splashes fall back into the molten steel pool.

Ingot mold coatings also provide other advantages, such as extending the life of the mold, facilitating the release of the ingot from the mold, and reduction of ingot surface imperfections.

Because of the manner in which steel ingots are formed, the demands on a mold coating are particularly stringent. The coating should be sufficiently fluid, so as to permit easy application to the mold, e.g., dipping or spraying. The composition must be relatively thermally stable at temperatures of up to 1200° F. and rapidly decompose or volatilize at 1900° F. The coating should result in little, if any, flaking or ashing. In addition, the coating should adhere well to the ingot mold surface and provide a relatively uniform coating on the surface.

**Description of the prior art**

U.S. Patent Nos. 520,076 and 1,752,725 teach the use of tars and bituminous materials as ingot mold coatings. In an article in the Proceedings of Open Hearth Steel Conference, 1962, p. 326, by Mr. J. F. Georgiadis, at p. 332, the use of Gilsonite and uncharacterized petroleum derivatives is taught for mold coating.

**2****SUMMARY OF THE INVENTION**

Excellent mold coatings are provided comprising from about 35 to 65 weight percent of an aromatic bitumen with, respectively, from about 65 to 35 weight percent of an aromatic lubricating oil extract wherein the final composition has an autoignition temperature in excess of at least 1100° F. and a combined asphaltene-aromatics to paraffin weight ratio of at least 3:1.

**DESCRIPTION OF THE PREFERRED EMBODIMENTS**

The ingot mold compositions of this invention combine about 35 to 65 parts of an aromatic bitumen with about 65 to 35 parts of an aromatic lubricating oil extract, more usually from about 40 to 60 parts to about 60 to 40 parts, respectively.

In combining the bitumen and the lubricating oil extract, any method which achieves homogeneity may be used. Usually, elevated temperatures will be employed to lower the viscosity.

The final composition has a kinematic viscosity at 180° F. in the range of about 400 to 1,700 cst. (centistokes), more usually 400 to 1,000 cst. When practicable, the kinematic viscosity may be as low as 300 cst.

25 The autoignition temperature of the mold coating composition is in excess of at least 1100° F. and will generally be in the range of 1150° F. to 1400° F. The autoignition temperature is determined as follows: A pyrometer is connected to a test plate and the temperature of the test plate raised to the desired temperature. Samples weighing 0.25 g. are placed in a steel cup (0.5" high and 0.75" in diameter), and the cup is then positioned on the test plate. By repeating the test upon the sample and a standard at various temperatures and noting temperature differences at which autoignitions occur, the autoignition temperature of the test sample can be determined.

30 The COC (Cleveland Open Cup) flash temperature is at least 425° F. and usually in the range of about 450° to 550° F. The test procedure is ASTM D92-57.

35 A further desirable property is to have a post-ignition temperature of at least 1100° F. and preferably at least about 1150° F. The post-ignition temperature indicates whether the mold coating may ignite after the mold has been placed on a stool. The test is carried out as follows: 40 The mold coating (0.25 g.) is weighed into a steel cup  $\frac{3}{8}$ " in diameter and 1" high, simulating the initial coating. The cup is placed for 45 seconds on a hot plate having a surface temperature of about 900° F. The cup is then put into a muffle furnace and the door closed to  $\frac{1}{4}$ ". 45 The furnace wall temperature is metered, and the temperature is recorded at which the mold ignites, the temperature of the muffle furnace being successively raised.

50 The mold coating composition will analyze to a weight ratio of the combined weight of asphaltenes and aromatics to paraffins of at least 3:1 and more usually at least 4:1. Preferably, the ratio will be at least 5:1 and may range from 10-100:1. The asphaltene content will be at least 15% and will generally not exceed 95 weight percent, more usually being in the range of about 20 to about 90 weight percent. The aromatics will be at least 5 weight percent and generally not exceed 70 weight percent, more usually being in the range of about 10 to about 55 weight percent.

Small amounts of other materials may also be present in the mold coating composition, either to enhance desirable properties of the composition or to provide new properties for the composition. Illustrative of such additives are fire retardants, antioxidants, water, phosphates and antifoaming agents. Usually, these additives will not exceed 10 weight percent of the total composition and more usually not exceed 5 weight percent of the total composition.

#### BITUMEN COMPONENT

As already indicated, the ingot mold composition has two major components: bitumen and a lubricating oil extract.

Generally, the bitumen will be derived from petroleum tar or pitch bottoms, usually obtained from thermal cracking (residua). Other sources of the bitumen may be used, as they provide the necessary properties.

The bitumen will have a penetration in the range of about 0 to 15, more usually 0 to 12 (ASTM D5-61). The bitumen is further characterized by having a softening point in the range of about 120 to 160, more usually in the range of about 135 to 155 (ASTM Method D36-26).

The composition of the bitumen will have at least 20 weight percent asphaltenes and may have as high as 95 weight percent asphaltenes, more usually in the range of about 25 to 90 weight percent asphaltenes. The paraffinics will be less than 25 weight percent and preferably less than about 20 weight percent. The ratio of the combined weight of asphaltenes and aromatics to paraffinics should be at least about 3:1 and preferably in the range of about 5-100:1. The aromatic or naphthenics (also called cycls) will generally be in the range of about 5 to 60 weight percent, more usually in the range of about 10 to 50 weight percent.

#### LUBRICATING OIL EXTRACT

The lubricating oil extract which is used is derived by the extraction of lubricating oil distillate with any one of a variety of solvents, e.g., propane, furfural, cresylic acid, sulfur dioxide, etc. The raffinate thus obtained is rich in paraffinics, while the extract is rich in aromatics, e.g., maltenes. Generalized descriptions of extraction procedures may be found in U.S. Patent Nos. 2,783,162 and 2,879,219.

The extract's composition will be as follows: at least 25 weight percent, and more usually in the range of about 30 to 98 weight percent, aromatics; paraffinics will generally be less than 10, and more usually less than 5 weight percent.

The kinematic viscosity at 140° F. of the lubricating oil extract will be in the range of about 100 to 200 cst., while the boiling range of the extract will be in the range of about 550° to 1000° F.

#### ILLUSTRATIVE EXAMPLES

In order to demonstrate the effectiveness of the compositions of this invention as ingot mold coatings, two samples were prepared having the following properties and compositions:

|                                   | I           | II          |
|-----------------------------------|-------------|-------------|
| Bitumen A, wt. percent.....       | 60          | .....       |
| Bitumen B, wt. percent.....       | .....       | 60          |
| Oil extract, wt. percent.....     | 40          | 40          |
| Autoglowing ° F.....              | 1,175-1,200 | 1,175-1,200 |
| Flash, C.O.C., ° F.....           | 475         | 460         |
| Fire point, ° F.....              | 510         | 515         |
| Vis. at 180° F., cst.....         | 747         | 1698        |
| Component analysis, wt. percent:* |             |             |
| Paraffins.....                    | 23.8        | 8.2         |
| Asphaltenes.....                  | 20.3        | 47.9        |
| Cycls (aromatics).....            | 55.9        | 43.9        |

\*The component determination is carried out as follows:

A 1.5 to 2.0 g. sample is weighed in a 250 ml. flask and 100 ml. of n-pentane added. A condenser is fitted to the flask, which is then placed in a water bath maintained at about reflux temperature (approximately 115° F.), allowing just the neck of the flask to remain above the surface. At the end of two hours, the flask is removed from the water bath and allowed to cool to room temperature, maintaining the condenser in place.

The above materials were tested in order to determine their utility as ingot mold coating compositions. The compositions were placed on a heated plate and maintained at that temperature for about one hour and the 5 percent weight loss determined. The percent weight loss is considered an indication of the coating performance of the subject mold coating.

In a second series of tests, the materials were heated for one hour at a prescribed temperature, then ignited at 10 1900° F. and the total weight loss determined to determine the volatile matter. The second step involving ignition at 1900° F. and determining the percent lost is considered to represent the volatile matter available during the pouring of the molten metal.

15

TABLE I

|                                                                      | Temperature, ° F. |      |         |      |         |      |
|----------------------------------------------------------------------|-------------------|------|---------|------|---------|------|
|                                                                      | 300° F.           |      | 500° F. |      | 700° F. |      |
| Example.....                                                         | I                 | II   | I       | II   | I       | II   |
| Percent loss after heating for one hour.....                         | 0.1               | 0.0  | 0.5     | 0.8  | 26.8    | 15.1 |
| Percent loss on ignition (1,900° F.) after heating for one hour..... | 85.0              | 81.4 | 82.4    | 79.1 | 42.5    | 55.8 |
| Total percent volatile matter.....                                   | 85.1              | 81.4 | 82.9    | 79.9 | 69.3    | 70.9 |

20

It is evident from the above table that a major proportion of the coating is retained on the metal surface for long periods of time at elevated temperatures, providing a protective coating for the mold and permitting easy release and the absence of irregularities and defects upon removal of the steel ingot from the mold.

A field test was carried out at a steel mill using ingot molds maintained at temperatures in the range of about 700° F. to 800° F. The composition of Example I was 35 tested and found not to flash when applied, to be readily applied by spraying and to provide a relatively smooth, even coating which was retained for long periods of time without flaking or significant ashing.

Three other ingot mold coating compositions were prepared and tested under field conditions in steel mills. These compositions were found to be readily applied to the ingot mold, not to flash or post-ignite, and to provide minimal amounts of imperfections and scabs on the ingot because of contacting of splashes with the mold. The following 45 table indicates the composition of the bitumen used, properties of the bitumen, properties of the lubricating oil extract, the ratio of materials used, and finally, the properties and analysis of the mold composition.

50

Mats are prepared for Gooch crucibles by mixing a small amount of asbestos fiber in water to form a suspension and then pouring the suspension through the crucible, followed by applying suction to the crucible until a mat of from about 0.5 to 1 mm. thickness is formed. The mat is then dried at 250° F. and weighed after cooling to room temperature in a desiccator.

The content of the flask is then filtered through the crucible, the flask being washed with three 10 ml. portions of n-pentane which are also filtered. The filtrate and washings are then transferred to a weighed 55 250 ml. beaker and 10 ml. of n-pentane used to wash the flask and make the transfer quantitative. The Gooch crucibles are then dried in an oven at 250° F., while the flasks used in the original extraction are cautiously heated on a hot plate to remove the bulk of adsorbed n-pentane and then placed into a 250° F. oven for 30 minutes. The flask and crucible are removed from the oven, cooled in a desiccator and weighed.

The above method provides a separation of asphaltenes from cycls and paraffinics. The combined weight of material retained in the extraction flask and crucible is the weight of asphaltenes reported. This procedure is analogous to that disclosed in Kleinschmidt, L. R., J. Research Natl. Bur. Standards, 54(3), 163 (1955).

The beaker containing the filtrate is cautiously heated until all the pentane has evaporated. The beaker is then cooled in a desiccator and weighed. Acetone is added, 35 ml. of acetone being used for each gram of pentane solubles. The beaker is then placed on a hot plate, covered with a watch glass and allowed to slowly reflux for 10 minutes. At the end of this time, the beakers are allowed to cool at room temperature and then placed in a freeze chest at -10° F. for from 16 to 18 hours. The liquid portion is then transferred to a tared beaker, and the solid residue rinsed with two 15 ml. portions of cold acetone (-10° F.), the washings being added to the transferred supernatant liquid. The acetone is evaporated on a hot plate and the beaker dried in a 250° F. oven to constant weight. The material dissolved in the acetone is reported as cycls (resins), while the residue is reported as paraffinics (oils). Duplicate samples can be carried out to check the results. The above method for separating paraffinics from cycls is analogous to that disclosed by Traxler, R. N., and Scheyer, H. E., Oil Gas J., 52 158 (1953).

(In reporting component percents throughout the specification, the 75 above procedure was used.)

TABLE II

|                                            | III   | IV    | V     |
|--------------------------------------------|-------|-------|-------|
| Composition, wt.:                          |       |       |       |
| Bitumen, percent.....                      | 58    | 55    | 65    |
| Oil extract, percent.....                  | 42    | 45    | 35    |
| Properties of mold coating composition:    |       |       |       |
| Viscosity at 180° F., est.....             | 465   | 495   | 485   |
| Autoignition, ° F.....                     | 1,150 | 1,200 | 1,250 |
| Post-ignition.....                         | 1,150 | 1,175 | 1,250 |
| Flash, C.O.C., ° F.....                    | 460   | 455   | 450   |
| Fire point, ° F.....                       | 510   | 510   | 505   |
| Component analysis:                        |       |       |       |
| Asphaltenes, percent.....                  | 24    | 55    | 54.2  |
| Aromatics, percent.....                    | 56    | 43.4  | 44.8  |
| Paraffins, percent.....                    | 20    | 1.0   | 1.0   |
| Coating test, 1 hr. at 800° F.:            |       |       |       |
| Visual, percent.....                       | 65    | 80    |       |
| Weight retained, percent.....              | 32    | 38    |       |
| Volatility, preliminary loss at:           |       |       |       |
| 500° F., percent.....                      | 3.5   | 2.1   |       |
| 700° F., percent.....                      | 41.4  | 25.8  |       |
| Ignition at 1,900° F., total loss:         |       |       |       |
| 500° F. conditioned.....                   | 78.4  | 78.4  |       |
| 700° F. conditioned.....                   | 70.2  | 65.2  |       |
| Properties of bitumen, component analysis: |       |       |       |
| Asphaltenes, percent.....                  | 33    | 94.8  | 90.1  |
| Aromatics, percent.....                    | 42    | 5.1   | 9.8   |
| Paraffins, percent.....                    | 25    | 0.1   | 0.1   |
| Autoignition, ° F.....                     | 1,275 | 1,325 | 1,325 |
| Flash, C.O.C., ° F.....                    | 500   | 495   |       |
| Softening point, ° F.....                  | 135   | 156   | 143   |
| Penetration at 77° F.....                  | 12    | ----- | 0     |
| Viscosity at 275° F., cst.....             | 240   | ----- | 735   |
| Properties of extract:                     |       |       |       |
| Viscosity at 140° F., cst.....             | 123   | 123   | 123   |
| Flash, C.O.C., ° F.....                    | 440   | 440   | 440   |
| Autoignition, ° F.....                     | 1,100 | 1,100 | 1,100 |
| Component analysis:                        |       |       |       |
| Asphaltenes, percent.....                  | 0.0   | 0.0   | 0.0   |
| Aromatics, percent.....                    | 98.0  | 98.0  | 98.0  |
| Paraffins, percent.....                    | 2.0   | 2.0   | 2.0   |

The above data effectively demonstrate that under laboratory and field conditions the compositions of this invention are excellent coatings for ingot molds protecting against irregularities and providing improved results in the coating.

Moreover, the mold coating compositions of this invention may be used in the preparation of ingots of other metals, e.g., copper. The mold coating compositions have been demonstrated to be capable of retaining coatings at elevated temperatures for long periods of time under stringent testing and may therefore be employed with a variety of molds and in the forming of ingots of metals other than iron.

As will be evident to those skilled in the art, various modifications on this invention can be made or followed, in the light of the foregoing disclosure and discussion, without departing from the spirit or scope of the disclosure or from the scope of the following claims.

## I claim:

1. An improvement in the method of preparing metal ingots using an ingot mold at a temperature of at least 500° F. which comprises coating the ingot mold prior to the pouring of the metal with a composition having the following properties: a kinematic viscosity at 180° F. of at least about 300 cst.; an autoignition temperature of at least 1,100° F.; a COC flash temperature of at least 425° F.; and, a weight ratio of asphaltene and aromatic components to the paraffinic component of at least 3:1; and,

wherein from 35 to 65 weight percent of said composition is derived from bitumen of from about 0 to 15 penetration and from about 120 to 160 softening point and having less than 25 weight percent paraffinics and greater than 20 weight percent asphaltenes; and respectively, 65 to 35 weight percent of an aromatic lubricating oil extract having at least 25 weight percent aromatics and less than 10 weight percent paraffinics and having a kinematic viscosity at 140° F. in the range of about 100 to 200 cst.

2. A method according to claim 1 wherein said metal is steel and wherein the ingot is used up to a temperature of about 1,200° F.

3. A method according to claim 1 wherein the weight ratio of asphaltene and aromatic components to the paraffinic component is in the range of 10-100:1.

4. A method according to claim 1 wherein the coating composition has an autoignition temperature in the range of about 1,150° to 1,400° F., and a kinematic viscosity at 180° F. in the range of about 400 to 1,700 cst.

5. A method according to claim 4 wherein the weight ratio of the asphaltene-aromatic components to the paraffinic component is at least 5:1.

## References Cited

## UNITED STATES PATENTS

|           |        |                 |            |           |
|-----------|--------|-----------------|------------|-----------|
| 1,752,725 | 4/1930 | Braden          | -----      | 106—38.25 |
| 2,308,245 | 1/1943 | Ortynsky.       |            |           |
| 2,783,162 | 2/1957 | Mollring        | -----      | 106—278   |
| 2,879,219 | 3/1959 | Benedict et al. | 106—279 XR |           |
| 3,096,192 | 7/1963 | Pitchford       | -----      | 106—281   |

45 JULIUS FROME, Primary Examiner.

L. B. HAYES, Assistant Examiner.

U.S. Cl. X.R.

117—168; 106—38.25, 278; 164—72